

Patented Jan. 15, 1935

1,987,639

# UNITED STATES PATENT OFFICE

1,987,639

## LEADED BRASS AND PROCESS OF MAKING IT

Robert T. Roberts, Riverside, Ill., assignor to  
Western Electric Company, Incorporated, New  
York, N. Y., a corporation of New York

No Drawing. Application November 12, 1931,  
Serial No. 574,677

15 Claims. (Cl. 75—1)

This invention relates to a leaded brass and a process of working such a brass and more particularly to a process of hot rolling leaded brass.

An object of the invention is to provide a leaded brass and an effective and efficient process of working such a brass.

It has been known for some time that brass consisting of about 60 to 63 per cent copper and 37 to 40 per cent zinc may be hot rolled at temperatures ranging from 1150° to 1600° F. This brass is known as yellow brass and on account of its tendency to crack upon slight corrosion, it has found but limited use in this country. Higher grades of brass, that is those containing a greater amount of copper, could heretofore, as far as can be learned, be hot rolled only when they were substantially free from lead and even then the temperature range at which the rolling could take place was limited to 1550° to 1650° F.

20 In accordance with one embodiment of the present invention, a small amount of silicon is added to a high grade brass which permits it to be hot rolled without edge cracking or breaking up during the hot rolling process.

25 On account of the fact that brass containing .03 per cent of lead or less is difficult to obtain and expensive, and also because even high grade brass containing .03 per cent or less of lead can be hot rolled only in a narrow temperature range, the general method of working brass has been to cast the brass in strips or sheets of 1.125 to 1.25 inches in thickness and then working the brass to smaller dimensions by alternately cold rolling and annealing. A certain amount of cold rolling of brass invariably results in embrittling the brass and, therefore, it must be annealed before further reduction in size can take place.

30 It has been found that by adding silicon in small amounts, ranging from .5 per cent to 1.5 per cent, to a high grade brass containing from 64 to 70 parts of copper and from 30 to 36 parts of zinc, the brass thus obtained may be rolled at a temperature range of 1150° to 1600° F. without edge cracking or breaking up even though the alloy 35 may contain lead as high as .5 per cent of the alloy. If a greater amount than .5 per cent of lead is present in the brass, this may be offset by adding 2 per cent or more of silicon. However, larger quantities of silicon than this have an undesirable effect upon the brass.

35 In practicing the invention in the preferred form, copper and brass are melted in the proportion of about 67 per cent copper and 32.5 per cent zinc to which 1/2 per cent silicon is added. The 40 resulting alloy may then be cast in ingots or slabs

of about 2 1/2 to 3 inches in thickness. These slabs are then hot rolled at a temperature from about 1150° to 1600° F. to a thickness of 1/4 inch in a single hot rolling operation.

The casting of the brass in slabs from 2 1/2 to 3 inches in thickness avoids a large amount of waste due to surface flaws in the slabs, since a thinner slab will have substantially the same amount of surface waste which is usually milled off.

45 Due to the fact that slabs having a thickness of 2 1/2 to 3 inches may be hot rolled to a thickness of 1/4 inch by following the process of this invention, the expense of alternately cold rolling and annealing is saved. After the slabs have been hot rolled to a thickness of 1/4 inch, they may be cold rolled without previous annealing because the hot rolling leaves the brass in an annealed condition.

50 This process makes it possible to use either new brass or scrap brass, such as salvaged from discarded telephone equipment, which usually contains a considerable amount of lead, or scrap brass may be added in any proportion to new brass. The addition of the silicon appears not only to offset the effect of the presence of lead in the alloy but high grade brass, which is substantially free from lead, may be hot rolled through a much wider temperature range, thereby facilitating the hot rolling operation.

55 It will be understood that the nature and embodiment of the invention herein described is merely an illustrative form of the invention and many changes and modifications may be made therein without departing from the spirit and scope of the invention.

What is claimed is:

1. A process of producing a brass alloy containing lead up to .5% which comprises adding silicon up to 2% of the alloy to render the brass capable 40 of being hot-rolled.

2. A brass capable of hot working, comprising approximately 60% to 70% of copper, substantial amounts of lead up to .50%, silicon up to 1 1/2%, and the balance approximately all zinc.

3. A brass capable of hot rolling, comprising approximately 63% to 70% of copper, substantial amounts of lead up to .5%, silicon up to 1 1/2%, and the balance approximately all zinc.

4. A brass capable of hot rolling, comprising 50 approximately 60% to 70% of copper, at least .5% lead, a substantial amount of silicon up to 2% to retain the hot rolling properties of the brass in the presence of said lead, and the balance approximately all zinc.

5. A brass capable of hot working, comprising approximately 63% to 70% of copper, at least .5% lead, a substantial amount of silicon up to 2% to retain the hot working properties of the brass in the presence of said lead, and the balance approximately all zinc. 5
6. A free cutting brass capable of hot working, comprising approximately 60% to 70% of copper, a small amount of lead, silicon in sufficient quantity to retain the hot working properties of the brass in the presence of said lead, and the balance approximately all zinc. 10
7. A free cutting brass capable of hot rolling, comprising approximately 63% to 70% of copper, a small amount of lead, silicon in sufficient quantity to retain the hot rolling properties of the brass in the presence of said lead, and the balance approximately all zinc. 15
8. A brass capable of hot working, comprising approximately 60% to 70% of copper, a small amount of lead, a substantial amount of silicon up to 2% to retain the hot working properties of the brass in the presence of said lead, and the balance approximately all zinc. 20
9. A brass capable of hot rolling, comprising approximately 63% to 70% of copper, a small amount of lead, a substantial amount of silicon up to 2% to retain the hot rolling properties of the brass in the presence of said lead, and the balance approximately all zinc. 25
10. Free cutting leaded brasses capable of hot rolling and drawing containing approximately from 60 to 70% copper, substantial amounts of lead up to 5%, substantial amounts of silicon up to 1.5%, and the balance approximately all zinc. 5
11. Leaded brasses capable of hot rolling containing approximately from 60 to 70% copper, substantial amounts of lead not exceeding 3%, substantial amounts of silicon not exceeding 2%, and the balance approximately all zinc. 5
12. Leaded brasses capable of hot rolling containing approximately from 60 to 70% copper, substantial amounts of lead not exceeding slightly more than .5%, substantial amounts of silicon not exceeding 2%, and the balance approximately all zinc. 10
13. Leaded brasses capable of hot rolling containing approximately from 60 to 70% copper, small amounts of lead, substantial amounts of silicon not exceeding 2% to retain the hot rolling properties of the brass in the presence of said lead, and the balance approximately all zinc. 15
14. A process of producing a brass alloy containing small amounts of lead, which comprises adding up to 2% of silicon to the alloy to neutralize the detrimental effect of the lead on the brass. 20
15. Leaded brasses capable of hot working containing approximately 60 to 70% copper, substantial amounts of lead not exceeding about 4%, substantial amounts of silicon not exceeding about 2%, and the balance approximately all zinc. 25

ROBERT T. ROBERTS.